

# United States Patent [19]

Nomura et al.

[11] 4,023,987

[45] May 17, 1977

[54] **METHOD OF PRODUCING SOFT THIN STEEL SHEET BY CONTINUOUS ANNEALING**

[75] Inventors: **Giichiro Nomura**, Kudamatsu; **Takuo Ando**, Yokohama; **Keiji Ariga**, Kudamatsu; **Akira Ikeda**, Kudamatsu; **Kinji Saito**, Kudamatsu; **Taizo Sato**, Kudamatsu, all of Japan

[73] Assignee: **Toyo Kohan Co., Ltd.**, Japan

[22] Filed: **Dec. 10, 1975**

[21] Appl. No.: **639,608**

[30] **Foreign Application Priority Data**

Dec. 20, 1974 Japan ..... 49-145750

[52] **U.S. Cl.** ..... **148/12 D**; **148/12 F**; **148/134**; **148/143**; **148/36**

[51] **Int. Cl.<sup>2</sup>** ..... **C21D 9/48**

[58] **Field of Search** ..... **148/12 C**, **12 D**, **12 F**, **148/12.3**, **36**, **134**, **143**

## [56] References Cited

### UNITED STATES PATENTS

|           |         |                      |          |
|-----------|---------|----------------------|----------|
| 3,806,376 | 4/1974  | Toda et al. ....     | 148/12 C |
| 3,839,095 | 10/1974 | Kubotera et al. .... | 148/12 C |
| 3,920,487 | 11/1975 | Gondo et al. ....    | 148/12 C |

### FOREIGN PATENTS OR APPLICATIONS

|           |        |              |          |
|-----------|--------|--------------|----------|
| 2,107,640 | 2/1971 | Germany .... | 148/12.3 |
|-----------|--------|--------------|----------|

*Primary Examiner*—Arthur J. Steiner  
*Attorney, Agent, or Firm*—Wenderoth, Lind & Ponack

## [57] ABSTRACT

A continuous annealing process for producing a soft tin plate and black plate with T - 2½ or T - 3 tempering properties is attained in a conventional continuous annealing furnace for black plate by the use of a novel steel strip composition.

**6 Claims, 6 Drawing Figures**

FIG.1



FIG.2



FIG. 3



FIG. 4





## METHOD OF PRODUCING SOFT THIN STEEL SHEET BY CONTINUOUS ANNEALING

### BRIEF SUMMARY OF THE INVENTION

The present invention relates to a method of producing a soft low carbon thin steel sheet and especially relates to a method of producing soft tin plate and black plate. In particular, the present invention relates to a continuous annealing process to produce a soft tin plate and black plate with T - 2½ or T - 3 tempering properties from a novel steel strip composition. It had previously been considered impossible to fabricate such products by a conventional continuous annealing furnace for black plate, and therefore such products have heretofore been produced by a box annealing process.

### BRIEF DESCRIPTION OF THE DRAWINGS

The drawings are described as follows:

FIG. 1 is a diagram of a conventional continuous annealing line which is commercially used to anneal the steel strip for tin plate and black plate.

FIG. 2 shows three examples of schematic diagrams for continuous annealing heat cycle for tin plate and black plate.

FIG. 3 is a diagram showing the relation between [Mn]/S in steel strips and the Rockwell 30T hardness of tin plate products.

FIG. 4 is the diagram showing the relation between phosphorus content of steel strip and Rockwell 30T hardness of tin plate products.

FIG. 5 is a diagram showing the relation between soaking temperature and the Rockwell 30T hardness of tin plate products in heat cycle with overaging.

FIG. 6 is a diagram showing the relation between the cooling rate before arriving at the overaging temperature and the Rockwell 30T hardness of tin plate products.

### BACKGROUND OF THE INVENTION

There are two type of annealing processes for the annealing of cold rolled low carbon steel strip. One is a continuous annealing process and the other is a box annealing process.

The continuous annealing process was originally developed, and has been used in Japan and other countries mainly to produce the steel strip for tin plate and black plate.

Tin plate and black plate are used for various purposes and their tempering properties are selected according to the demands of various finished articles.

In section 5 of JIS (Japanese Industrial Standard) G 3303-1969 (hereinafter referred to as "JIS") "Tin plate and Black plate", the temper of tin plate and black plate is designated by numerical value of the Rockwell 30T hardness (HR 30T) and it is also remarked that "the term 'temper' when applied to tin plate and black plate can not essentially be represented by any single mechanical property. However, the Rockwell 30T hardness test value is chosen as one of the most effective guide of interrelated mechanical properties".

Furthermore, in A 623-1973 of the ASTM (American Society for Testing and Materials) Standard (hereinafter referred to as "ASTM"), the term "temper" is defined as follows: "7.1 Single-Reduced Tin Mill Product, Temper-the term temper when applied to single-

reduced tin mill products summarizes a combination of interrelated mechanical properties. No single mechanical test can measure all the various factors which contribute to the fabrication characteristics of the material.

The Rockwell 30T hardness value has come into general use as a quick test which serves as a guide to the properties of the plate.

The temper of "tin plate and black plate" is designated by a numerical value of the Rockwell 30T hardness and this numerical value serves as a guide to the production of tin plate and black plate. The temper ranges of tin plate and black plate, represented by the Rockwell 30T hardness value, at which the producer should aim, are classified into seven JIS classifications as shown in Table I. The classification of the temper in the ASTM scheme is similar to that of Table I but T - 2½ is not included in the ASTM scheme.

In Table I, temper T - 1 and T - 2 are extremely soft and therefore are utilized where severe forming conditions are to be encountered. Temper T - 4, T - 5, T - 6, T - 4 - CA, T - 5 - CA, T - 6 - CA are utilized when stiffness and hardness of tin plate or black plate is especially required.

Tin plate with temper T - 2½ and T - 3 properties are most suitable for normal can body and end use as well as for various other purposes. Therefore the demand for T - 2½ and T - 3 material is the greatest.

TABLE I

| The temper of tin plate under JIS standards |            |                              |            |
|---------------------------------------------|------------|------------------------------|------------|
| Box annealing process                       |            | Continuous annealing process |            |
| Temper designation                          | Aim HR 30T | Temper designation           | Aim HR 30T |
| T - 1                                       | 49±3       |                              |            |
| T - 2                                       | 53±3       |                              |            |
| T - 2½                                      | 55±3       |                              |            |
| T - 3                                       | 57±3       |                              |            |
| T - 4                                       | 61±3       | T - 4 - CA                   | 61±3       |
| T - 5                                       | 65±3       | T - 5 - CA                   | 65±3       |
| T - 6                                       | 70±3       | T - 6 - CA                   | 70±3       |

However, tin plate or black plate with temper T - 2½ or T - 3 properties has not yet been produced by a conventional continuous annealing process, and therefore has been produced by a box annealing process as can be seen from Table I.

The steel strip for black plate is cold rolled to a more than 80% reduction in thickness so that the steel strip after cold rolling is very hard, low in ductility and shows a fiber structure. Therefore it is necessary to anneal the cold rolled strip to recrystallize, cause grain growth, change the fiber structure into the granular structure, and give softness and workability to the steel strip.

In a box annealing process, coils of the steel strip are piled on one or several stacks within an inner cover filled with a slightly reducing gas atmosphere. The stack of coils in the inner cover is heated by a Bell-type heating furnace covering the inner cover and it takes several days to finish the box annealing heat cycle, i.e. the heating process, the soaking process and the cooling process.

The deformation of the steel strip and furthermore, annealing stickers sometimes occur during box annealing. These defects lead to the inferior shape of the steel strip and also to the low yield of the product.

Furthermore, box annealing products show a considerable heterogeneity in their mechanical properties because of the localized heat application and the non-uniformity of heat distribution within a coil and between coils. However, the long heating and soaking time in the box annealing cycle lead to an appropriately large grain size, and the long cooling time leads to a nearly complete precipitation of carbon and nitrogen from the ferrite matrix which had been dissolved in said matrix at the soaking temperature. Consequently the box annealed products are soft and have excellent formability as well as a quite low aging tendency due to its low carbon and nitrogen content in solution.

On the other hand, as shown in FIG. 1, the continuous annealing furnace for tin plate is divided into four main zones; heating zone 3, soaking zone 4, slow cooling zone 5 and fast cooling zone 6. A certain number of upper rolls and bottom rolls are provided in each zone. The cold rolled steel strip 8 is fed from the pay-off reel 1, cleaned in the cleaning section 2 in order to remove rolling lubricants and then runs through upper and bottom rolls in strands as shown in FIG. 1. Then the steel strip is recoiled by the recoiler 7 at room temperature after the whole cycle of heating, soaking, slow cooling and fast cooling. This whole process takes only a few minutes.

Throughout this annealing process the strip is protected from oxidation by a protective gas atmosphere. The products continuously annealed show uniform mechanical properties because of the uniformity of heat distribution in the steel strip. Furthermore the tension in the furnace section results in a product of superior shape, and the products can be produced in a short time by continuous annealing. However, grain growth in the course of recrystallization is not sufficient because of very short heating time and soaking time. Moreover, carbide and nitride do not precipitate sufficiently, almost all of these two elements, dissolved in ferrite matrix during the soaking period, remain in a supersaturated solid solution after annealing because of an extremely short cooling time compared with that of box annealing. Consequently continuously annealed steel strip is sufficient in strength but is slightly lacking in workability and inevitably shows aging phenomena because of the two above-mentioned causes.

Type MR steel and Type MC steel are known as representative raw materials for tin plate and black plate in JIS. Cast chemical compositions of Type MR and MC steels are shown in Table II.

TABLE II

| Chemical composition of base metal steel |      |      |      |       |       |
|------------------------------------------|------|------|------|-------|-------|
| Base-metal<br>Steel type                 | C    | Si   | Mn   | P     | S     |
| MR                                       | 0.13 | 0.01 | 0.60 | 0.020 | 0.050 |
| MC                                       | 0.13 | 0.01 | 0.70 | 0.150 | 0.050 |

Type MR steel is a normal low carbon steel, and Type MC steel is a low carbon steel rephosphorized in order to increase its strength. In a box annealing process, black plate with temper T - 1, T - 2, T - 2½ or T - 3 is usually produced from Type MR material.

On the other hand, black plate with temper T - 4, T - 5 or T - 6 is usually produced from Type MC steel or Type MR steel renitrogenized with 0.007% nitrogen minimum. A continuous annealing process is suitable for the production of black plate having good stiffness together with high strength. In a continuous annealing

process, type MC steel or Type MR steel renitrogenized with 0.007% nitrogen minimum is used to produce the black plate with temper T - 6 - CA or T - 5 - CA, and Type MR steel is used to produce the black plate with temper T - 5 - CA or T - 4 - CA. However, it has not yet been possible to produce black plate with temper T - 2½ or T - 3 by a conventional continuous annealing process.

Recently new techniques have been developed to apply the continuous annealing process to the production of normal cold rolled steel sheet for thicker gauges than tin plate.

In these new developments, the steel strip is so constituted as to be given a special treatment, i.e. holding at some intermediate temperature after or in the course of cooling from the recrystallization temperature, to promote the precipitation of carbon which was dissolved into the iron matrix at the recrystallization temperature for the promotion of softening of the iron matrix. This treatment for the promotion of softening by the precipitation of carbides is referred to as "overaging treatment" or "shelf-treatment".

For instance, in laid-open Japanese patent application No. Sho 49-35218, a method is described to produce the low carbon steel strip having low yield strength, high Lankford's *r* value, and good conical cup value by a continuous annealing process.

The raw materials suitable for this purpose should contain low manganese ( $\leq 0.30$ ), low nitrogen ( $\leq 20$  ppm) and also satisfy the following formula:

$$O \leq (Mn\%) - \frac{\text{atomic weight of Mn}}{\text{atomic weight of O}} \times (0\%)$$

$$- \frac{\text{atomic weight of Mn}}{\text{atomic weight of S}} \times (S\%) \leq 0.15.$$

Then the hot steel strip is coiled at high temperature i.e.  $600^\circ - 800^\circ$  C after hot-strip rolling, heated and soaked to produce recrystallization and then undergoes the overaging treatment in a continuous annealing line after cold-rolling. German Offenlegungsschrift 2064487 has the same claims as the laid-open Japanese patent application No. Sho 49-35218 but has a restriction of Mn = 0.25% and no restriction of nitrogen.

In the second example thereof, Japanese patent publication No. Sho 49-1968 is described as follows: the cold rolled low carbon steel strip is rapidly cooled to below  $200^\circ$  C with a cooling rate of more than  $20^\circ$  C/sec when the soaking temperature is lower than the  $A_1$  point. When the soaking temperature is higher than the  $A_1$  point, the cold rolled low carbon steel strip is slow cooled to just below the  $A_1$  point with the cooling rate of less than  $20^\circ$  C/sec and then rapidly cooled to below  $200^\circ$  C with a cooling rate of more than  $20^\circ$  C/sec. After rapid cooling, the cold rolled low carbon steel strip is re-heated to an overaging temperature and kept at this temperature for a few minutes, (3 - 5 minutes in the examples). A low carbon steel strip having low yield strength and excellent elongation is obtained by this method.

As a third example, in laid-open Japanese patent application No. Sho 47-26313, a carbon steel ingot ( $0.02\% \leq C \leq 0.10\%$ ) is rolled to form a slab, is hot-strip rolled and is coiled at normal temperature or at a higher temperature (above  $630^\circ$  C), and then is cold rolled. The cold rolled low carbon steel strip is

heated to a temperature between the recrystallization temperature and 850° C in the continuous annealing furnace, and then is slowly cooled to a temperature ranging between 600° C and near the  $A_1$  point, and then is rapidly cooled to room temperature with the cooling rate of 200° C/sec - 10,000° C/sec. The steel strip rapidly cooled to room temperature is re-heated to a temperature between 300° C and 530° C and is kept for more than 10 seconds at this temperature. The low carbon steel sheet having excellent drawability and low aging properties can be efficiently produced by this continuous annealing process and its properties in drawability and aging is described to be equal to or better than that of the box annealed product.

The newly developed special continuous annealing methods mentioned above enables the fabrication of a soft steel strip with excellent workability by continuous annealing. However, these methods will be expensive because it is necessary to observe several restrictions including overaging treatment. Moreover, the continuous annealing equipment becomes complicated and the length of the total line becomes very long compared with the length of the conventional continuous annealing line for tin plate and black plate.

The several restrictions mentioned above are as follows:

1. A severe limitation concerning the composition of the steel is necessary.
2. Hot-coiling at considerably higher temperature after hot-strip rolling is required.
3. "Overaging treatment" is necessary.
4. Overaging time is long.
5. Rapid cooling prior to the overaging treatment is necessary.

Furthermore, the steel strip for tin plate and black plate is very thin, and therefore the reduction in cold rolling is more than 80% even when thin hot-rolled steel strip (2.0 mm thick) is used. Consequently, the steel strip for tin plate or black plate is somewhat inferior in workability after annealing to a normal cold rolled steel sheet which is cold rolled with a 60 - 70% reduction.

After annealing, black plate is temper rolled and electroplated in the electrolytic tinning line followed by subsequent heating to above 232° C in the "flow brightening" process. Also in the case of hot-dip tinning, black plate is dipped into the molten tin where the temperature is more than 300° C. In other words, after annealing, the steel strip is strained and then heated during the fabrication process of tin plate. Therefore the tin plate products are strain-aged and hardened, and consequently its workability is inferior to the "as annealed state".

Thus, it is difficult to produce an extremely soft tin plate having temper T - 1 or T - 2 properties even by the newly developed continuous annealing process for thicker steel sheet mentioned above with the conventional low carbon steel strip.

According to the Journal of the Iron and Steel Institute of Japan, Volume 60 (1974) No. 4, S,331, the coldrolled Type MR steel strip for tin plate (0.32 mm thick), reduced with the reduction of more than 80% was annealed under continuous conditions disclosed in laid-open Japanese patent application No. Sho 47-26313, temper rolled with an elongation of 1.5%, and then artificially aged by a heat cycle similar to "flow-brightening" in the electrolytic tinning process.

A product having temper T - 2 1/2 was consequently obtained.

Therefore it became clear that these new continuous annealing processes for the thicker cold rolled steel strip utilizing overaging treatment made it only possible to fabricate tin plate as soft as temper T - 2 1/2 at best.

#### DETAILED DESCRIPTION OF THE INVENTION

With the process of the present invention, it is possible to produce soft tin plate and black plate having temper T - 3 or T - 2 1/2 with a slight but feasible restriction concerning the composition of type MR steel (JIS). Type MR steel is widely used as the most suitable raw material for tin plate and black plate.

15 The continuous annealing cycle used includes a conventional continuous annealing cycle for tin plate stock, hereinafter referred to as the first embodiment or a slightly modified continuous annealing cycle utilizing a short overaging treatment, hereinafter referred to as the second embodiment.

In the present invention, coiling at high temperature after hot-strip rolling is not necessarily required and a very long furnace for overaging is unnecessary because a short overaging treatment provides sufficient softening, and it is possible to use a conventional continuous annealing line for tin plate and black plate without any remodeling. Therefore the present invention is very useful for continuously annealing the steel strip for tin plate and black plate.

25 30 In the following, we explain the present invention in detail. Three typical examples of continuous annealing cycle are shown in FIG. 2. The normal continuous annealing furnace for tin plate is divided into four main zones; a heating zone, a soaking zone, a slow cooling zone and a fast cooling zone as shown in FIG. 1.

The total length of the steel strip stored in each zone is calculated from three factors; the diameters of the top and bottom rolls, the distance from the top rolls to the bottom rolls and the number of passes (number of strands).

40 45 A practical annealing cycle in a specific continuous annealing line is determined by the temperature in each zone, the operating speed and the length of the cold rolled steel strip stored in each zone.

The ratio of seconds, in which the steel strip passes through the above said four zones, is constant and independent of the operating speed of the continuous annealing line.

50 55 The cycle A in FIG. 2 shows an annealing cycle in a conventional industrial continuous annealing line utilized for tin plate and black plate (this line is hereinafter referred to as No. 1 CAL) with the following conditions, soaking temperature: 730° C, operating speed: 366 m/min (1200 fpm). This No. 1 CAL has a heating zone with 10 passes, a soaking zone with 8 passes, a slow cooling zone with 10 passes and a fast cooling zone with 10 passes.

In the operation shown as the cycle A in FIG. 2, the steel strip is heated from room temperature (point a in FIG. 2) to 730° C in 25 seconds during its passage through the heating zone (point b in FIG. 2), is soaked at this temperature for 20 seconds (point c in FIG. 2), slow cooled to 480° C in 25 seconds (point d in FIG. 2), at the cooling rate of 10° C/sec and is then fast cooled to room temperature in 25 seconds (point e in FIG. 2). In this cycle, it takes about 20 seconds to cool from 550° to 250° C, and the total annealing time is 95 seconds.

This No. 1 CAL is operated commercially within the speed range of from 458 m/min (1500 fpm) to 305 m/min (1000 fpm), and the corresponding cooling time from 550° to 250° C is from 16 seconds to 24 seconds respectively, and the total time for annealing is from 76 seconds to 114 seconds respectively.

A normal continuous annealing cycle for black plate falling within the scope of the first embodiment of this invention, has the following characteristics; (1) the total time is within 2 minutes and (2) the time needed to cool from 550° to 250° C is within 30 seconds. The cycle A shown in FIG. 2 is a typical example of this category.

The cycle C in FIG. 2 shows an annealing cycle in another industrial continuous annealing line for tin plate and black plate (this line is hereinafter referred to as No. 2 CAL) with the following conditions, soaking temperature: 707°- 715° C, operating speed: 183 m/min (600 fpm). This line has a heating zone with 8 passes, a soaking zone with 8 passes, a slow cooling zone with 12 passes and a fast cooling zone with 12 passes. In the operating condition of the cycle C shown in FIG. 2, the steel strip is heated from room temperature (point a in FIG. 2) to 707° C (point b' in FIG. 2) in 38.8 seconds during its passage through the heating zone, is soaked or slow heated to 715° C (point c' in FIG. 2) for 38.8 seconds, is slow cooled to 507° C (point d' in FIG. 2) in 58.4 seconds and then is fast cooled to room temperature in 58.8 seconds (point e' in FIG. 2). In this cycle, it takes about 44 seconds to cool from 550° to 250° C, and the total annealing time is 194.8 seconds. If this No. 2 CAL is operated at the speed of 244 m/min (800 fpm), it will take about 33 seconds to cool from 550° to 250° C, with the total annealing time of 146.1 seconds.

It became clear from above examples that the annealing cycle in which the cooling time from 550° to 250° C requires over 30 seconds and can be obtained by reducing the operating speed of the normal continuous annealing line for tin plate and black plate. The cycle C in FIG. 2 is representative.

The cycle B shown in FIG. 2 is another example, falling within the scope of what will be referred to as the second embodiment of this invention. This cycle B is obtained in a model testing apparatus for continuous annealing operation. In this modeling testing apparatus, it is also possible to obtain cycle A or cycle C shown in FIG. 2 by changing components in the line and the testing speed.

In the operating conditions for cycle B, the steel strip is heated from room temperature (point a in FIG. 2) to 800° C (point b' in FIG. 2) in 26 seconds, is soaked at this temperature for 26 seconds (point c' in FIG. 2), is cooled to 450° C in 35 seconds at the cooling rate of 10° C/sec (point d' in FIG. 2), is overaged at 450° C for 60 seconds (point e' in FIG. 2) and then is cooled to room temperature in 45 seconds (point f in FIG. 2).

In cycle B, it takes about 91 seconds to cool from 550° to 250° C and the total annealing time is 192 seconds.

To practice this overaging in a commercial continuous annealing line, it is necessary to change the design and alignment of zones in the annealing line, i.e. to introduce an overaging zone between the slow cooling zone and final fast cooling zone. It takes only 30-60 seconds, however, to achieve effective overaging in the present invention, therefore it is unnecessary to install a long overaging zone in the line. This superiority leads

to the reduction of both the construction cost and the operating cost. The cycle B shown in FIG. 2 is the representative annealing cycle that satisfies the objectives of the second embodiment of this invention, including a comparatively short overaging treatment.

In the following, the cold rolled steel strip of various compositional ranges was annealed by the cycle A, cycle B, cycle C and other similar cycles within the invention. The tests were made by using both the model testing apparatus and the industrial continuous annealing lines for tin plate and black plate. The steel strip after annealing was temper rolled by 1.5%, electrolytically tinned in an acid sulphate bath and then flow-brightened (heated to above the melting point of tin) to bring the steel strip to a fully aged state. Sample discs are cut from the steel strips, and their Rockwell 30T hardness was tested using the Rockwell T superficial hardness tester.

FIG. 3 shows the relation between the Rockwell 30T hardness (Rockwell T superficial hardness: HR 30T) of tin plate products and the value of  $\{(Mn\%) - (55/16)(0\%) \} / (S\%)$  (this formula is hereinafter referred to as [Mn]/S) calculated from the compositions of the steel strip of a low carbon rimmed or capped steel strip.

Zone A in FIG. 3 depicts the Rockwell 30T hardness of the tin plate manufactured by cycle A (in FIG. 2) wherein its carbon content  $\leq 0.05\%$ , manganese content  $\leq 0.50\%$ , nitrogen content  $\leq 0.0030\%$  and phosphorus content  $\leq 0.012\%$ . Zone B in FIG. 3 depicts the Rockwell 30T hardness of the tin plate manufactured by cycle B (in FIG. 2) with its carbon content  $\leq 0.10\%$ , manganese content  $\leq 0.50\%$ , phosphorus content  $\leq 0.020\%$  and nitrogen content  $\leq 0.0030\%$ . In the relationship

$$[Mn]/S = \{(Mn\%) - (55/16)(0\%) \} / (S\%)$$

(Mn%), (0%) and (S%) are weight percent of manganese, oxygen and sulphur contained in the steel strip respectively, and [Mn] is the quantity of manganese in the steel strip that is able to combine with sulfur to form manganese sulfide. The broken line X, Y corresponds to the center values of temper T - 3 and T - 2½, respectively.

As shown in FIG. 3, a clear correlation between the Rockwell 30T hardness of tin plate and the value of [Mn]/S can be recognized in both zone A and zone B. With an increase in the value of [Mn]/S, the Rockwell 30T hardness is reduced. In the range where [Mn]/S  $\geq 20$  in zone A, the upper limits of distributed results satisfy the temper T - 3 grade, and so it becomes possible to produce soft tin plate having temper T - 3 properties from this material. In the range where [Mn]/S  $< 12$  in zone B, the Rockwell 30T hardness is rather high and its distribution is considerably scattered. Therefore it is necessary to establish the restriction "[Mn]/S  $\geq 12$ " in order to insure the tin plate products possess temper T - 2½ or T - 3 properties, taking the segregation of the compositions in the steel strip into account.

Comparing zone A with zone B, zone B is found to be 2 or 3 points softer in the Rockwell 30T hardness than zone A, because of the effect of overaging treatment. Therefore the restriction of [Mn]/S in zone B is less than the one in zone A. Points 3a and 3b in FIG. 3 depict the Rockwell 30T hardness of tin plate with 0.009% vanadium in the cycle A of FIG. 2 and in the cycle B of FIG. 2 respectively. Points 4a and 4b in FIG. 3 depict the Rockwell 30T hardness of tin plate with

0.19% chromium in the cycle A of FIG. 2 and in the cycle B of FIG. 2 respectively. From these results it is clear that a small amount of carbide forming element in the steel is sufficiently effective in case of the cycle A of FIG. 2, where the Rockwell 30T hardness is 2 - 3 points softer compared with normal steel without special elements and shows the same superior softening effect as in case of the cycle B of FIG. 2.

5

From the viewpoint of softening steel strips, the higher soaking temperature is favorable, but the upper limit of soaking temperature is restricted to 900°C in consideration of the type of furnace and convenience in operation. As shown in this example, a whole range of temper T - 2½ properties can be realized when proper heat cycles are selected within the scope of the second embodiment of this invention.

Table III

| type of steel | Chemical composition of the steel (%) |      |      |       |       |       |        |        |
|---------------|---------------------------------------|------|------|-------|-------|-------|--------|--------|
|               | C                                     | Si   | Mn   | P     | S     | O     | N      | [Mn]/S |
| rimmed        | 0.048                                 | 0.01 | 0.40 | 0.013 | 0.019 | 0.021 | 0.0025 | 17     |

In FIG. 4 the relation between the phosphorus content and the Rockwell 30T hardness of tin plate is shown. Zone A is the Rockwell 30T hardness of tin plate produced by the cycle A of FIG. 2 with carbon content  $\leq 0.05\%$ , manganese content  $\leq 0.50\%$ , the 20 value of  $[Mn]/S \geq 20$  and nitrogen content  $\leq 0.0030\%$ . Zone B is the Rockwell 30T hardness of tinplate produced by the cycle B of FIG. 2 with carbon content  $\leq 0.10\%$ , manganese content  $\leq 0.50\%$ , sul-

20

25

30

35

40

45

50

55

60

65

70

75

80

85

90

95

100

105

110

115

120

125

130

135

140

145

150

155

160

165

170

175

180

185

190

195

200

205

210

215

220

225

230

235

240

245

250

255

260

265

270

275

280

285

290

295

300

305

310

315

320

325

330

335

340

345

350

355

360

365

370

375

380

385

390

395

400

405

410

415

420

425

430

435

440

445

450

455

460

465

470

475

480

485

490

495

500

505

510

515

520

525

530

535

540

545

550

555

560

565

570

575

580

585

590

595

600

605

610

615

620

625

630

635

640

645

650

655

660

665

670

675

680

685

690

695

700

705

710

715

720

725

730

735

740

745

750

755

760

765

770

775

780

785

790

795

800

805

810

815

820

825

830

835

840

845

850

855

860

865

870

875

880

885

890

895

900

905

910

915

920

925

930

935

940

945

950

955

960

965

970

975

980

985

990

995

1000

1005

1010

1015

1020

1025

1030

1035

1040

1045

1050

1055

1060

1065

1070

1075

1080

1085

1090

1095

1100

1105

1110

1115

1120

1125

1130

1135

1140

1145

1150

1155

1160

1165

1170

1175

1180

1185

1190

1195

1200

1205

1210

1215

1220

1225

1230

1235

1240

1245

1250

1255

1260

1265

1270

1275

1280

1285

1290

1295

1300

1305

1310

1315

1320

1325

1330

1335

1340

1345

1350

1355

1360

1365

1370

1375

1380

1385

1390

1395

1400

1405

1410

1415

1420

1425

1430

1435

1440

1445

1450

1455

1460

1465

1470

1475

1480

1485

1490

1495

1500

1505

1510

1515

1520

1525

1530

sulphur content in the first embodiment at  $\leq 0.025\%$ , considering the balance of steel quality and the cost needed to remove sulphur from molten steel with some suitable means.

Lower nitrogen content is preferred too, but we restrict the nitrogen content in the first embodiment to  $\leq 0.0030\%$  considering the use of normal low carbon MR steel strip. The manganese content in the steel strip is restricted to  $\leq 0.50\%$  in the first embodiment by the same reason. The oxygen content in the steel strip reduces the value of the expression  $(\text{Mn}\%)-(55/16) \times (0\%)$ , and deteriorates the value of  $[\text{Mn}]/\text{S}$  consequently; therefore it is desirable to reduce the oxygen content as low as possible. In the case of the second embodiment, it is impossible to fabricate soft tin plate, since the Rockwell 30T hardness of tin plate products increases when the carbon content is more than 0.10%.

With regard to the sulphur, manganese and nitrogen content, we restrict these as follows in the second embodiment for the same reasons as in the first embodiment.

$$\text{S} \leq 0.025\%, \text{Mn} \leq 0.50\% \text{ and N} \leq 0.0030\%.$$

Concerning the oxygen content in the second embodiment, it is desirable to lower it so as not to deteriorate the value of the expression  $(\text{Mn}\%)-(55/16) \times (0\%)$ .

As for the phosphorus content, the Rockwell 30T hardness of tin plate is reduced sufficiently by the restriction of  $\text{P} \leq 0.015\%$  even if the value of  $[\text{Mn}]/\text{S}$  is smaller than 12 as shown in the following example 1 (refer to sample No. 12, No. 13 and No. 14 in Table V and Table VI).

Therefore, it is only necessary to employ normal type MR steel (JIS) with the additional restriction of either  $[\text{Mn}]/\text{S} \geq 12$  or  $\text{P} \leq 0.015\%$  in case of the second embodiment.

Some tin plate samples in FIG. 3 or FIG. 4 also fluctuate to have a temper T - 2½ or T - 3 grade, despite being slightly outside the scope of this invention. But in order to insure the tin plate products possess temper T - 2½ or T - 3 properties, taking the segregation of the compositions in the steel strip into account, the restric-

tions for the compositions of the steel strip must be as mentioned above.

Concerning the steel types, rimmed or capped steel produced by the top-blown oxygen converter process is desirable. In the fabrication of capped steel ingot, it is desirable to minimize the oxygen content contained in the steel.

Open-hearth steel is not preferred because it is impossible to remove the impurities originating from the scrap and also, open-hearth steel has a higher nitrogen content, resulting in the Rockwell 30T hardness of tin plate produced by open-hearth steel being much higher.

However, steel fabricated by any other processes can be used, if similar to the clean steel produced by the top-blown oxygen process.

The following Examples are representative but not limitative of the present invention.

#### EXAMPLE 1

Rimmed or capped steel was rolled from an ingot into a slab, hot rolled into hot band of 2 mm thickness, cold rolled after pickling to 0.32 mm (cold reduction 84%), and continuously annealed by the cycle A or the cycle B shown in FIG. 2, temper rolled at a 1.5% elongation, electrolytically tinned, and then, the surface tin was flow-brightened. The compositions of the steel strip employed are shown in Table V. Both the Rockwell 30T hardness after annealing and the Rockwell 30T hardness of tin plate product are shown in Table VI.

The analyses of sample Nos. 1 to 8 satisfy both first and second embodiments, showing temper T - 3 properties via cycle A of FIG. 2 and temper T - 2½ properties via cycle B of FIG. 2.

Sample Nos. 9 and 10, the analyses of which satisfy neither first nor second embodiment, show temper T - 4 or the upper value of T - 3 properties via cycle B of FIG. 2.

Sample Nos. 11 to 14, which satisfy the steel composition of the second embodiment, show temper T - 4 properties via cycle A of FIG. 2, but temper T - 2½ or T - 3 properties via cycle B of FIG. 2.

TABLE V

| Chemical composition of the steel ( % ) |            |       |      |      |       |       |       |        |                        |       |       |
|-----------------------------------------|------------|-------|------|------|-------|-------|-------|--------|------------------------|-------|-------|
| sample No.                              | steel type | C     | Si   | Mn   | P     | S     | O     | N      | $[\text{Mn}]/\text{S}$ | Cr    | V     |
| 1                                       | rimmed     | 0.027 | 0.01 | 0.33 | 0.008 | 0.011 | 0.018 | 0.0014 | 24                     |       |       |
| 2                                       | rimmed     | 0.043 | 0.01 | 0.37 | 0.006 | 0.016 | 0.012 | 0.0022 | 21                     |       |       |
| 3                                       | rimmed     | 0.048 | 0.01 | 0.40 | 0.012 | 0.015 | 0.021 | 0.0025 | 22                     |       |       |
| 4                                       | rimmed     | 0.050 | 0.01 | 0.41 | 0.008 | 0.010 | 0.020 | 0.0025 | 34                     |       |       |
| 5                                       | rimmed     | 0.036 | 0.01 | 0.37 | 0.010 | 0.012 | 0.016 | 0.0023 | 26                     |       |       |
| 6                                       | rimmed     | 0.042 | 0.01 | 0.38 | 0.007 | 0.011 | 0.029 | 0.0025 | 25                     |       |       |
| 7                                       | rimmed     | 0.034 | 0.01 | 0.35 | 0.009 | 0.010 | 0.024 | 0.0024 | 27                     |       |       |
| 8                                       | rimmed     | 0.035 | 0.01 | 0.33 | 0.010 | 0.012 | 0.018 | 0.0010 | 22                     |       |       |
| 9                                       | capped     | 0.050 | 0.01 | 0.34 | 0.016 | 0.020 | 0.065 | 0.0024 | 6                      |       |       |
| 10                                      | rimmed     | 0.069 | 0.01 | 0.36 | 0.016 | 0.026 | 0.027 | 0.0039 | 10                     |       |       |
| 11                                      | rimmed     | 0.041 | 0.01 | 0.34 | 0.015 | 0.021 | 0.027 | 0.0028 | 12                     |       |       |
| 12                                      | capped     | 0.036 | 0.01 | 0.29 | 0.013 | 0.030 | 0.054 | 0.0017 | 3                      |       |       |
| 13                                      | rimmed     | 0.051 | 0.01 | 0.26 | 0.009 | 0.019 | 0.027 | 0.0026 | 9                      |       |       |
| 14                                      | capped     | 0.028 | 0.01 | 0.20 | 0.010 | 0.020 | 0.063 | 0.0023 | -1                     |       |       |
| 15                                      | rimmed     | 0.030 | 0.01 | 0.31 | 0.007 | 0.014 | 0.008 | 0.0027 | 20                     | 0.016 | 0.009 |
| 16                                      | rimmed     | 0.050 | 0.01 | 0.33 | 0.006 | 0.014 | 0.008 | 0.0014 | 22                     | 0.19  | 0.005 |
| 17                                      | capped     | 0.040 | 0.01 | 0.28 | 0.011 | 0.022 | 0.065 | 0.0026 | 3                      |       |       |
| 18                                      | capped     | 0.040 | 0.01 | 0.27 | 0.014 | 0.025 | 0.065 | 0.0024 | 2                      |       |       |

TABLE VI

| sample<br>No. | steel<br>type | [Mn]/S | P     | Chemical composition and hardness |                    |              |         |                                                                          |                                          |
|---------------|---------------|--------|-------|-----------------------------------|--------------------|--------------|---------|--------------------------------------------------------------------------|------------------------------------------|
|               |               |        |       | Rockwell 30 T hardness (HR 30T)   |                    |              |         | note                                                                     |                                          |
|               |               |        |       | cycle A                           | after<br>annealing | tin<br>plate | cycle B |                                                                          |                                          |
| 1             | rimmed        | 24     | 0.008 | 52.4                              | 57.6               | 48.1         | 54.6    |                                                                          |                                          |
| 2             | rimmed        | 21     | 0.006 | 52.7                              | 57.7               | 49.6         | 55.9    |                                                                          |                                          |
| 3             | rimmed        | 22     | 0.012 | 53.0                              | 58.0               | 50.4         | 55.4    |                                                                          |                                          |
| 4             | rimmed        | 34     | 0.008 | 52.9                              | 57.9               | 50.0         | 55.3    |                                                                          |                                          |
| 5             | rimmed        | 26     | 0.010 | 52.9                              | 58.7               | 49.3         | 55.2    | Satisfies first<br>and second embodi-<br>ments                           |                                          |
| 6             | rimmed        | 25     | 0.007 | 52.7                              | 57.7               | 48.6         | 54.8    |                                                                          |                                          |
| 7             | rimmed        | 27     | 0.009 | 53.3                              | 59.5               | 49.5         | 54.7    |                                                                          |                                          |
| 8             | rimmed        | 22     | 0.010 | 52.8                              | 58.1               | 48.2         | 54.3    |                                                                          |                                          |
| 9             | capped        | 6      | 0.016 | 56.1                              | 61.2               | 53.3         | 58.8    | Departs from first<br>and second embodiments                             |                                          |
| 10            | rimmed        | 10     | 0.016 | 55.5                              | 61.3               | 54.0         | 59.6    |                                                                          |                                          |
| 11            | rimmed        | 12     | 0.015 | 55.0                              | 60.5               | 50.6         | 56.0    |                                                                          |                                          |
| 12            | capped        | 3      | 0.013 | 55.8                              | 61.1               | 50.1         | 55.6    |                                                                          |                                          |
| 13            | rimmed        | 9      | 0.009 | 53.4                              | 60.5               | 51.2         | 56.7    | Satisfies second<br>embodiment<br>vanadium<br>added<br>chromium<br>added |                                          |
| 14            | capped        | -1     | 0.010 | 54.7                              | 61.5               | 52.5         | 57.4    |                                                                          |                                          |
| 15            | rimmed        | 20     | 0.007 | 53.3                              | 56.6               | 49.6         | 55.8    |                                                                          |                                          |
| 16            | rimmed        | 22     | 0.006 | 53.8                              | 55.2               | 51.2         | 55.8    |                                                                          |                                          |
| 17            | capped        | 3      | 0.011 | 54.2                              | 61.0               | 52.5         | 57.6    | coiled at normal<br>temperature (680° C)                                 |                                          |
| 18            | capped        | 2      | 0.014 | 55.3                              | 60.4               | 51.7         | 56.4    |                                                                          | coiled at higher<br>temperature (680° C) |

Sample No. 15 contains vanadium and sample No. 16 contains chromium. The addition of vanadium or chromium is especially effective in cycle A of FIG. 2. They show temper T - 2½ properties even in the cycle A although the value of [Mn]/S by analysis is at the lowest range permitted in the first embodiment.

Sample No. 17 and No. 18 which satisfy the second embodiment show the effect of coiling temperature after hot rolling of strip. Increasing the coiling temper-

25 raus contents of these two samples are less than 0.015% to satisfy the second embodiment but the values of [Mn]/S of these steels are small, and therefore the values of the Rockwell 30T hardness remains at the upper range of temper T - 3.

Concerning the overaging time at 450° C, 60 seconds is considered to be enough because there can be seen little change in the Rockwell 30T hardness after 60 seconds.

TABLE VII

| Chemical composition of the steel (%) |               |       |      |      |       |       |       |        |        |                            |
|---------------------------------------|---------------|-------|------|------|-------|-------|-------|--------|--------|----------------------------|
| sample<br>No.                         | steel<br>type | C     | Si   | Mn   | P     | S     | O     | N      | [Mn]/S | note                       |
| 1                                     | capped        | 0.045 | 0.01 | 0.30 | 0.011 | 0.017 | 0.065 | 0.0022 | 5      | coiling<br>temp.<br>600° C |
| 2                                     | capped        | 0.039 | 0.01 | 0.29 | 0.008 | 0.015 | 0.060 | 0.0020 | 6      | coiling<br>temp.<br>600° C |

TABLE VIII

| Overaging time and hardness (HR 30T) |      |       |                    |              |                    |              |                    |              |                    |              |
|--------------------------------------|------|-------|--------------------|--------------|--------------------|--------------|--------------------|--------------|--------------------|--------------|
| sample<br>No.                        | Mn/S | P     | 30 seconds         |              | 60 seconds         |              | 300 seconds        |              | /800 seconds       |              |
|                                      |      |       | after<br>annealing | tin<br>plate | after<br>annealing | tin<br>plate | after<br>annealing | tin<br>plate | after<br>annealing | tin<br>plate |
| 1                                    | 5    | 0.011 | 54.1               | 59.8         | 53.4               | 58.7         | 52.0               | 57.8         | 52.3               | 58.6         |
| 2                                    | 6    | 0.008 | 53.0               | 58.9         | 52.3               | 57.7         | 52.1               | 58.2         | 51.7               | 57.8         |

ture from 600° C to 680° C results in a tendency towards reduced Rockwell 30T hardness in case of both the cycle A and the cycle B of FIG. 2.

55

## EXAMPLE 3

The compositions of the steel strip used are shown in Table VII. The steel was rolled from an ingot to a slab, hot rolled into hot band of 2.0 mm thickness, pickled and cold rolled to a steel strip 0.32 mm thick, and then continuously annealed in cycles similar to cycle B of FIG. 2 in which 30, 60, 300 and 1800 seconds at 450° C were selected as overaging treatment, temper rolled to 1.5% in elongation, and electrolytically tinned and flow-brightened.

The results of the Rockwell 30T hardness measurement of tin plate are shown in Table VIII. The phospho-

60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 67

tion of its operating speed, even if the carbon content of steel strip is higher than 0.05%.

TABLE IX

The result of continuous annealing test  
(cycle C of FIG. 2)

| sample<br>No. | steel<br>type | C    | Si   | Mn   | P     | S     | O     | N      | hardness (HR 30 T) |                    |              |
|---------------|---------------|------|------|------|-------|-------|-------|--------|--------------------|--------------------|--------------|
|               |               |      |      |      |       |       |       |        | [Mn]/S             | after<br>annealing | tin<br>plate |
| 1             | capped        | 0.07 | 0.01 | 0.33 | 0.013 | 0.017 | 0.030 | 0.0022 | 13                 | 52.0               | 56.3         |
| 2             | capped        | 0.06 | 0.01 | 0.32 | 0.013 | 0.013 | 0.028 | 0.0024 | 17                 | 52.5               | 56.8         |

## EXAMPLE 4

Two rimmed steel ingots were rolled into slabs, hot rolled into hot bands of 2.0 mm thickness, of which the compositions are listed in Table X, pickled and cold rolled to 0.32 mm thick, continuously annealed by the cycle B of FIG. 2, temper tolled to 1.5% in elongation, and then electrolytically tinned and flow-brightened.

The Rockwell 30T hardness and other mechanical properties measured as shown in Table XI. The Rockwell 30T hardness of the sample No. 1 showed the center value of T - 2½ range and that of the sample No. 2 showed the center value of T - 3 range.

Other mechanical properties also proved to be equal to the ones of usual box-annealed products, showing low yield strength and ultimate tensile strength together with excellent elongation.

On the other hand, the desirable lower limits of chromium and vanadium added are 0.02% and 0.005% respectively in order to provide a sufficient number of carbide nuclei to serve as targets or sites for the diffusion and precipitation of carbon atoms.

The Rockwell 30T hardness of products are reduced with increasing soaking temperature when continuously annealed in a cycle satisfying the second embodiment of the present invention, and show the lowest value of temper T - 2½ range, i.e. 52 - 53 (HR 30T) at the soaking temperature of 900°C.

Coiling at higher temperature after hot rolling of strip has a slight effect on the softening of continuously annealed products, but the difficulty in descaling in the pickling of the hot strip before cold rolling is a drawback of higher-temperature-coiled products, sometimes resulting deterioration of surface appearance of

TABLE X

Chemical composition of the steel (%)

| Sample<br>No. | Steel<br>type | C     | Si   | Mn   | P     | S     | O     | N      | [Mn]/S |
|---------------|---------------|-------|------|------|-------|-------|-------|--------|--------|
| 1             | rimmed        | 0.024 | 0.01 | 0.28 | 0.007 | 0.011 | 0.036 | 0.0008 | 14     |
| 2             | rimmed        | 0.036 | 0.01 | 0.34 | 0.015 | 0.022 | 0.029 | 0.0010 | 11     |

TABLE XI

Mechanical properties  
(tin plate produced by a practical annealing line)

| sample<br>No. | hardness (HR 30 T)<br>after<br>annealing | yield<br>strength<br>Kg/mm <sup>2</sup> | tensile<br>strength<br>Kg/mm <sup>2</sup> | elongation<br>(%) | work<br>hardening<br>modulus (n) | Lankford's<br>value(r) | note |
|---------------|------------------------------------------|-----------------------------------------|-------------------------------------------|-------------------|----------------------------------|------------------------|------|
| 1             | 48.6                                     | 54.7                                    | 28.4                                      | 35.3              | 36.0                             | 0.16                   | 1.31 |
| 2             | 52.4                                     | 57.5                                    | 32.1                                      | 37.9              | 30.6                             | 0.15                   | 1.25 |

As mentioned above in detail, proper restriction of the amount of carbon, manganese, sulphur, nitrogen and phosphorus in the steel strip together with the value of [Mn]/S make it possible to fabricate continuously annealed soft tinplate with temper T - 3 properties in case of the cycle A of FIG. 2 and with temper T - 2½ or T - 3 properties in case of the cycle B or cycle C of FIG. 2 where the time to cool from 550°C to 250°C is longer than 30 seconds.

The addition of a trace of carbide former such as 60 chromium or vanadium, is quite effective in the softening, and in particular, the addition of these carbide formers strengthens the effectiveness of the cycle A of FIG. 2 up to the level of the cycle B of FIG. 2, which contains an overaging step.

Concerning the amount of chromium or vanadium, the desirable upper limits of chromium and vanadium are 0.20% and 0.03% respectively, considering the

tin mill products. Therefore coiling at high temperature is not necessarily required.

As has been explained, it is unnecessary to apply any particular treatment in the processes of ingot processing, slab rolling and hot-strip rolling to practice the present invention. Therefore the present invention is a superior industrial method for fabrication of soft tin plate having temper T - 2½ or T - 3 properties with high productivity by simple apparatus.

What is claimed is:

1. A method of producing a soft thin steel sheet in a continuous annealing heat cycle for tin plate and black plate with T-2½ or T-3 tempering properties which consists of:
  - a. heating a steel strip to a soaking temperature ranging from the recrystallization temperature to 900°C by a continuous annealing furnace, without an overaging zone, used in annealing black plate,

- b. maintaining said heat soaking temperature for 16 to 48 seconds,
- c. cooling to about 550° C in 20 to 60 seconds,
- d. cooling from 550° C to 250° C within 30 seconds and
- e. cooling to room temperature in 16 to 48 seconds, said steel strip being that produced by rolling a rimmed or capped steel ingot to form a slab, hot-strip rolling, and cold rolling to form a steel strip, the composition of said steel strip consisting essentially of: C  $\leq$  0.050%, Mn  $\leq$  0.50%, S  $\leq$  0.025%, N  $\leq$  0.0030%, P  $\leq$  0.012%,  $\{(Mn\%) - (55/16)(0\%)\}/(S\%) \geq 20$ , Fe and inevitable residual impurities.

2. A method of producing a soft thin steel sheet in a continuous annealing heat cycle for tin plate and black plate with T - 2½ or T - 3 tempering properties which consists of:

- a. heating a steel strip to a soaking temperature ranging from recrystallization temperature to 900° C,
- b. maintaining said heat soaking temperature for 20 to 48 seconds,
- c. cooling to about 550° C at the cooling rate of less than 20° C/sec,

d. cooling from 550° C to 250° C in more than 30 to 91 seconds or maintaining a temperature ranging from 550° to 250° C for more than 30 6 seconds and less than 60 seconds, and then cooling to room temperature,

said steel strip being that produced by rolling a rimmed or capped steel ingot to form a slab, hot-strip rolling, and cold rolling to form a steel strip, the composition of said steel consisting essentially of C  $\leq$  0.10%, Mn  $\leq$  0.50%, S  $\leq$  0.025%, P  $\leq$  0.020%, N  $\leq$  0.0030%, Fe and inevitable residual impurities, and satisfying at least one condition of the following two conditions;

- a. P  $\leq$  0.015% and
- b.  $\{(Mn\%) - (55/16)(10\%)\}/(S\%) \geq 12$ .
- 3. A method according to claim 1 wherein the steel strip additionally contains 0.02 to 0.20% chromium or 0.005 to 0.03% vanadium by weight.
- 4. A method according to claim 2 wherein the steel strip additionally contains 0.02 to 0.20% chromium or 0.005 to 0.03% vanadium by weight.
- 5. The soft thin steel sheet for tin plate and black plate produced by the process of claim 1.
- 6. The soft thin steel sheet for tin plate and black plate produced by the process of claim 2.

\* \* \* \* \*

30

35

40

45

50

55

60

65